

July 20, 1926.

1,593,058

E. BORNAND

SEALING BODY

Filed July 18, 1924

fig. 1.



fig. 2.



fig. 3.



fig. 4.



Witnessed by:  
elisabeth von Herrmann

R. Heimgartner

fig. 5.



Immunitor:  
Eduard Bornand

## UNITED STATES PATENT OFFICE.

ERNEST BORNAND, OF BERNE, SWITZERLAND.

## SEALING BODY.

Application filed July 18, 1924, Serial No. 726,870, and in Switzerland August 8, 1923.

Sealing wax usually used in sticks or lozenges is inconvenient in that it is necessary to have an appliance to heat it. They have already tried to do away with this inconvenience, for the sticks, by providing these with a wick of fibrous matter, like a candle, or with combustible fibrous material mixed with the composition, or with a real candle, but this did not act, as the wick or fibrous material does not provide sufficient heat to melt the mass of wax, so that it is the latter, which in burning gives the required heat to reduce the end of the stick to a semifluid state, that is applied to the object required to be sealed. This cannot be done without a slight carbonization and decomposition of the wax which is disagreeable and the operation takes too much time.

The sticks of sealing wax, provided with candles, are moreover very difficult to manufacture and it can happen, when they are being used, that melted paraffine or stearine gets mixed in with the sealing wax.

The employment of mixtures, containing more or less explosive material has also been suggested. Such mixtures are not suitable for sticks. On lozenges there will be left a quantity of ashes, which spoils the looks of the seal.

These disadvantages are done away with in the application of this invention. The sealing body made in accordance with the present invention is unique in that it consists of a piece of sealing wax having firmly held in contact therewith one or more pieces of a solid combustible material comprising in major part a solid and volatilizable polymerized aldehyde, so arranged that the combustible material can be easily ignited.

Such an aldehyde in practically pure state may be used, for instance, agglomerated through pressure, or it may be mixed with a small proportion of an agglomerating substance, as is explained further on.

We may advantageously employ, for example, metaldehyde ( $C_2H_4O$ )<sub>3</sub> or trioxymethylene ( $CH_2O$ )<sub>3</sub>. The metaldehyde is obtained through the polymerization of the acetaldehyde; it forms white crystals and burns without melting. Such bodies have the advantage to burn with sufficient rapidity and do not leave any ashes.

In the following it is understood that the combustible used is metaldehyde, but the invention is not limited to the use of this

body; and another polymerized solid and volatile aldehyde, for example, trioxymethylene, could also be used.

The wax can be in the form of sticks with a shaft of metaldehyde placed in the center, in the manner that graphite is placed in a pencil. This shaft may either be placed in the center or more or less out of center. The wax can also be made up in the form of lozenges either of one colour, or several colours, showing in their face side grooves in which is placed a small quantity of metaldehyde. The metaldehyde may also be simply laid on the wax. Each of the lozenges then already forms a little seal, which it will only be necessary to put on the required place and ignite. When the metaldehyde has burned, the wax has melted and the required impression may be made by the application of the seal. The upper part of the lozenges may with advantage be encased in a light celluloid shell or other covering which ignites easily, in order to instantly light the whole upper surface of the lozenge. This latter may also be in the form of an escutcheon.

Either the metaldehyde or the shell used in order to light it, or even the wax itself may have an aromatic substance, or liquid, added in order to give a perfume to the articles requiring to be sealed or to produce an agreeable odour when sealing. The composition of the wax may be the same as in ordinary sealing wax, or be made more easily fusible. The use of a wax which melts easily is made possible by the fact that there is no longer any fear that drops of wax fall on the object used to heat it (a candle for example) since this is done away with. The sealing body here described offers the many advantages enumerated below:

(1) Great convenience of application, resulting from the leaving away of a combustible substance, on the outside of the sticks or the lozenges.

(2) Great cleanliness: we can henceforth seal our letters without fear of soiling our hands.

(3) The colour of the seals obtained is the same as the colour of the wax employed, which is due to the fact that the wax, in this new process, is no longer brought to such high temperatures as to change its constituent elements, more especially its colour. It

follows that the seals made with this new wax are far more beautiful than the other ones.

(4) We obtain a reduction which ought 5 not to be neglected in the price of the wax through the fact that substances are left out, which in the ordinary kinds of wax are intended to keep up the combustion.

(5) The sealing body here described has 10 likewise great advantages from the fact that the wax is simply brought to the state of fusion and no longer to the point of combustion as is the case with ordinary wax, of eliminating the risk of burning the documents and securities contained in the letters 15 to be sealed, as sometimes happens with ordinary wax.

A wax giving good results may be made 20 for example of the following substances: Venetian turpentine 15 parts, black rosin 35 parts, gum lae 20 parts, plaster of Paris 30 parts, cinnabar 5 parts.

The annexed sketch gives an idea of the 25 two ways of working out the object of the invention.

Figure 1 shows an ordinary stick furnished with a shaft of metaldehyde.

Figures 2 and 3 are variations.

Figure 4 shows a lozenge seen from above. 30 Figure 5 shows a section of the same lozenge.

For the preparation of the sticks, they can 35 be per example formed by moulding in two lots, one of which shows a groove to receive a small shaft of metaldehyde and the other will attach itself to the surface formed by the wax and the metaldehyde, these parts being joined afterwards by the heat; another way may consist in running the wax 40 in fusion in the moulds with a core to keep the required place for the shaft of metaldehyde. It is better that the core may be displaced while the wax is cooling, in order to avoid any sticking. It is advantageous 45 to work with several moulds, that is to say showing several cavities for moulding placed parallel. The cores are formed of parallel strips extending from end to end of the mould and can be bound by a single 50 transverse bar, like the teeth of a comb. The movement of the cores may be made by a rotating cam working on the transverse bar and by a spring. Instead of allowing the movement of the cores during the cooling, it 55 is possible also after cooling, to rapidly reheat the cores with the object of melting the wax that had stuck to them and thus allow the cores to be removed. This could be done e. g. by passing an electric current, the cores making a conductor, or by furnishing these with an interior resistance 60 through which the current could pass. The cores could advantageously be in iron or other cheap metal to which the wax would stick as little as possible. The cores could

also be simply formed of hollow tubes through which we could pass a cooling fluid, in order to prevent the wax from sticking.

The insertion of the shafts of metaldehyde in the sticks can be executed by placing 70 these in the parallel grooves of a plate, grooves in the extension of which the holes of the sticks occur. Several shafts can thus be introduced at one and the same time by pushing them with the help of a movable 75 medium which will introduce sliding teeth into the grooves. The shafts of metaldehyde should form from a tenth to a twenty-fifth part of the stick. The same stick could contain two or more shafts of metaldehyde. 80

It may be advantageous, in order to ensure that the whole of the stick of wax can be made use of, to supply the end of the stick with a U-shaped handle in wood or other suitable material (see Fig. 2). 85

The lozenges could be produced through pouring or through stamping out of a still plastic mass of sealing wax. For the forming of the lozenges one could cover tablets of wax with a composition formed of metaldehyde in powder form mixed hot for preference, in a very highly concentrated solution of black rosin in alcohol. The quantity of the solution used and its concentration shall preferably be such, that the combustible material after hardening through evaporation of the alcohol, shall contain from 5 to 15% of black rosin. Such a composition could also be used to make the shafts to be put into the sticks. It is understood that under the expression "wax for sealing" we are to understand any and all substances which are convenient for sealing and have to be previously heated for the operation of sealing; "sealing wax" and "wax for sealing" do mean the same thing. 100

Having thus described my invention, what I consider is new and desire to secure by Letters Patent in the United States is:

1. A sealing body consisting of a piece 110 of sealing wax having firmly held in contact therewith at least one piece of a solid combustible material comprising in major part a solid and volatilizable polymerized aldehyde, so arranged that the combustible material can be easily ignited. 115

2. A sealing body, consisting of a piece of sealing wax having firmly held in contact therewith at least one piece of a solid combustible material substantially consisting of a solid and volatilizable polymerized aldehyde, so arranged that the combustible material can be easily ignited. 120

3. A sealing body consisting of a piece of sealing wax made in the shape of a stick, and of one shaft of a solid combustible substantially consisting of a solid and volatilizable polymerized aldehyde, the shaft being disposed within the stick of the wax as well as arranged longitudinally of the latter. 125 130

4. A sealing body consisting of a piece of sealing wax made in the shape of a stick and of one shaft substantially consisting of metaldehyde, the shaft being disposed within the stick of the wax as well as arranged longitudinally of the latter. 10
5. A sealing body consisting of a piece of sealing wax made in the shape of a stick and of one shaft substantially consisting of metaldehyde, the shaft being disposed within the stick of the wax as well as arranged longitudinally of the latter but away from the longitudinal center thereof.

In testimony whereof I affix my signature.

ERNEST BORNAND.